

1

2,947,692

## METAL DRAWING LUBRICANT

Everett C. Hughes, Shaker Heights, and Harrison M. Stine, Lyndhurst, Ohio, assignors to The Standard Oil Company, Cleveland, Ohio, a corporation of Ohio

No Drawing. Filed Nov. 9, 1956, Ser. No. 621,214

1 Claim. (Cl. 252—28)

The present invention relates to a method of drawing metals such as in the cold drawing of steel rods and the drawing of aerial bomb noses and to an improved lubricant for such operations.

Drawing involves the plastic deformation of metal by a hard steel die. High temperatures and pressures are generated between the die surface and the metal being drawn, and sufficient lubrication is required in order to prevent adhesion of the metal to the die surface and to prevent scratching and tearing of the surface of the drawn object. It is necessary for drawing fluids to cool the metal, reduce friction, and diminish seizure. Ease of application and removal of the drawing fluid from the surface of the metal are also important considerations.

Heretofore, mineral lubricants, fatty lubricants, soaps and waxes have been used to provide lubricating films for this type of operation, and a typical drawing compound of the prior art may include sulfurized olein, castor oil and sodium soap. Inert solid materials such as calcium carbonate have also been used as components of lubricating compositions designed for metal drawing operations and have proved to be of great value in forming a solid film between the metal and the die, thereby preventing metal to metal contact under high pressures.

Metal drawing compounds are customarily supplied to the trade as relatively viscous compositions some of which are intended to be diluted with oil and others to be diluted with water as dictated by the particular requirements in each mode of use. A drawing compound containing an inert solid material, such as calcium carbonate, which can be diluted satisfactorily with either oil or water is desirable. Such a compound must possess the following characteristics:

- (1) It must be capable of dilution with oil without settling of the inert solid material.
- (2) It must be capable of dilution with water and capable of holding the inert solid material in suspension.
- (3) It must remain the proper consistency when stored before dilution.

The drawing compounds of the prior art do not meet all of these requirements. While drawing compounds containing an inert solid material which are dilutable with oil have been provided, the problem of providing a composition of this type which is dilutable also with water has not been solved. Inert solid materials such as calcium carbonate are not readily suspending in water and the problem of obtaining a good suspension, in the case of a drawing compound, is complicated by the requirement that the drawing compound be dilutable also with oil. Another complicating factor is that the compound must be of suitable viscosity for dilution.

In accordance with this invention, there is provided a drawing compound which can be diluted with either oil or water to provide a highly satisfactory lubricant for drawing operations. The lubricants thus prepared provide both oiliness lubrication and solid film-type lubrication.

The drawing compounds of this invention are composed of four essential ingredients which are combined

2

in certain proportions to provide a formulation which meets all of the aforesaid requirements. The compositions include a suspended phase and a suspending phase. The suspended phase includes bentonite and an inert solid material having a hardness of 1-3.5 on Mohs' scale. The suspending phase includes a mineral lubricating oil and an emulsifying agent. The proportions of the ingredients must be so balanced that the suspended phase comprises from 60-75% by weight of the composition and the suspending phase from 40-25% by weight of the composition.

The mineral oil used in the formulation may be any mineral lubricating oil such as conventionally refined neutral oil, solvent extracted oil or any lubricating oil having a viscosity within the range of about 50 to about 500 Saybolt Universal seconds at 100° F. The mineral oil is generally the major ingredient of the suspending phase and may comprise from about 50-88% by weight of the suspending phase. The mineral oil serves a dual role in the composition. It is both a carrier for the inert solid material and it is an auxiliary lubricant.

The emulsifying agent can be any of those surface active agents which are commonly used in the preparation of emulsions, particularly oil-in-water emulsions, such as alkali metal, ammonium or hydroxylamine salts of fatty acids, petroleum sulfonates including long chain alkyl sulfates and alkyl-aryl sulfonates, polyoxyethylene derivatives of phenols, alcohols, etc., and the like. Preferred emulsifying agents are the sodium salts of petroleum sulfonic acids having molecular weights between 375 and 525. In addition to the emulsifying agent, emulsion stabilizers such as glue or gelatin may also be employed.

The amount of emulsifying agent is not critical. Any amount that emulsifies oil in water in the usual range of dilution intended for the drawing compound of this invention may be employed. Generally, it is preferred to employ from 12-50% of the emulsifying agent based on the weight of the suspending phase. When petroleum sulfonates are used as the emulsifying agent the maximum amount to be employed is limited by the viscosity to the composition, because petroleum sulfonates are relatively viscous materials. However, higher concentrations of petroleum sulfonates can be used with mineral oils in the lower part of the viscosity range given herein above.

Among the inert solid materials which may be used are those which are substantially insoluble in water or oil and have a hardness of 1 to 3.5 on Mohs' scale of hardness. Such substances include calcium carbonate, zinc sulfide, lithopone, talc, and other types of clay. The inert material is employed in finely divided form and is preferably fine enough to pass a 150 mesh screen.

A hydrophilic bentonite is employed to maintain the inert solid, such as calcium carbonate, in suspension in the suspending phase of the mixture, after dilution with water, as a result of the formation by the water and the bentonite of a thixotropic gel. The bentonite employed is preferably ground to a fine, odorless grit-free powder, having a particle size sufficiently small to pass a 200 mesh screen. For the purpose of this invention, it is necessary that the bentonite be in its natural state as in this state it is highly hydrophilic. Organophilic bentonites are not suitable for the purposes of this invention.

Bentonite and the inert solid material together comprise the suspended phase. The inert solid material comprises the major ingredient of the suspended phase and is preferably employed in amounts ranging from 85-97% by weight of the suspended phase and the bentonite in amounts ranging from 15-3% by weight of the suspended phase.

A most important factor in the compositions of this invention is the proportion of the suspending phase to

the suspended phase which is controlled by the consistency of the composition and its stability against separation into two phases. It has been found, for example, that a concentration of 75% by weight of the suspended phase is the maximum amount that can be tolerated to produce a composition with a workable consistency to permit ease of stirring. On the other hand, about 60% by weight of the suspended phase was found to be lower limit because compositions containing less solid matter evidenced separation of oil on prolonged standing.

The dilution of the drawing compound of this invention is limited only by the stability of the suspension of the solid material in the oil phase of the formulation. It has been found that the drawing compound may be diluted with several times its own weight of either oil or water or both. Generally, however, the degree of dilution will be controlled by the viscosity desired for the particular drawing operation to be performed.

A preferred lubricating composition consists of 18% by weight of conventionally refined neutral oil, 12% by weight of an oil-soluble sodium petroleum sulfonate of the mahogany acid type such as those available under the trade names "Petronate," "Petromix No. 9," and "Hardesty Base 19," 64% by weight of precipitated calcium carbonate, and 6% by weight of a natural bentonite.

The invention will be further illustrated by reference to the following specific examples:

#### EXAMPLE 1

One hundred pounds of a soluble oil consisting of 60% by weight of a conventionally refined neutral oil having a viscosity of 100 SUS at 100° F. and 40% by weight of an emulsifying agent composed of a sodium petroleum sulfonate having a molecular weight of about 450 were placed in a vessel. Two hundred ten pounds of precipitated calcium carbonate and 20 pounds of natural bentonite ground to pass a 200 mesh screen were slowly added to the soluble oil while agitating the mixture with a one-barrel size "Lightnin" mixer. A smooth creamy paste resulted.

The lubricating compound was diluted for use in a drawing operation with 1½ volumes of water per volume of drawing compound.

#### EXAMPLES 2 THROUGH 12

A series of formulations was prepared using the procedure and ingredients of Example 1. The proportions of ingredients and observations appear in the following table:

All of the compositions for which data are given in Table I have proved to be satisfactory. It is desirable

Table I  
[Wt. percent concentration of components]

| Example No.     | CaCO <sub>3</sub><br>(Ground),<br>150 mesh | Bentonite,<br>200 mesh | Emulsi-<br>fying Agent | Oil, C.R. Neutral                       | Dilution of 1 vol.<br>Mixture With |                                   | Stability vs. Separation on<br>Standing      |
|-----------------|--------------------------------------------|------------------------|------------------------|-----------------------------------------|------------------------------------|-----------------------------------|----------------------------------------------|
|                 |                                            |                        |                        |                                         | Vol. H <sub>2</sub> O              | Vol. Oil<br>(Diamond<br>Paraffin) |                                              |
| 2               | 67.0                                       | 6.3                    | 10.7                   | 16.0                                    |                                    |                                   | Desired consistency.                         |
| 3               | 67.0                                       | 6.3                    | 10.7                   | 16.0                                    | 1                                  |                                   | Very satisfactory (heavy cream consistency). |
| 4               | 67.0                                       | 6.3                    | 10.7                   | 16.0                                    |                                    |                                   | Satisfactory.                                |
| 5               | 67.0                                       | 6.3                    | 10.7                   | 16.0                                    |                                    |                                   | Satisfactory (easily dispersed).             |
| 6               | 66.9                                       | 6.4                    | 5.3                    | 21.4                                    | 1                                  |                                   | Very satisfactory (overnight bleeding).      |
| 7               | 66.9                                       | 6.4                    | 5.3                    | 21.4                                    |                                    |                                   | 16% bleeding (readily dispersed).            |
| 8               | 66.9                                       | 6.4                    | 5.3                    | 8.0 +13.4 S.E.<br>500 sec. <sup>3</sup> |                                    |                                   | 10% bleeding (readily dispersed).            |
| 9               | 66.9                                       | 6.4                    | 4.3                    | 22.4 S.E. 500 sec.<br>(3)               |                                    |                                   | 18% bleeding (readily dispersed).            |
| 10 <sup>2</sup> | 63.5                                       | 6.1                    | 12.2                   | 18.3                                    | 1                                  |                                   | Very satisfactory.                           |
| 11 <sup>2</sup> | 63.5                                       | 6.1                    | 12.2                   | 18.3                                    | 3                                  |                                   | Slight amount of carbonate at bottom.        |
| 12 <sup>2</sup> | 63.5                                       | 6.1                    | 12.2                   | 18.3                                    |                                    | 8                                 | Do.                                          |

<sup>1</sup> Percent bleeding after 72 hours standing.

<sup>2</sup> Precipitated calcium carbonate.

<sup>3</sup> 100 SUS at 100° F.

that the compositions prior to dilution have a viscous paste-like consistency so that they may be easily admixed with water or oil and this characteristic is possessed by the undiluted compositions of Examples 2, 7, 8, and 9. Similarly, it is desirable that the compositions, before dilution, be stable against separation of the two phases and this property also is possessed by the compositions of Examples 2, 7, 8, and 9. It should be noticed that bleeding is not a fatal defect if the compositions can be readily redispersed. Although some bleeding occurred in the compositions of Examples 7, 8, and 9, the compositions are nevertheless acceptable because they are readily redispersible.

After dilution, it is desirable that the diluted compositions have a consistency somewhat like that of heavy cream and all of the diluted compositions, i.e. Examples 3, 4, 5, 6, 10, 11, and 12, have this desired consistency. Similarly, the diluted compositions also must be stable against separation into two phases, i.e. a suspended phase and a suspending phase. All of the diluted compositions are satisfactory in this respect. It is noted that a slight amount of calcium carbonate precipitated to the bottom of the compositions of Examples 11 and 12 on standing. However, the amount of precipitate was so small as to be negligible and unobjectionable.

The examples adequately illustrate the adaptability of the compositions of this invention to dilution with either oil or water, giving the compositions a versatility that is not possessed by competitive products.

Tests of the lubricating compounds in drawing operations showed the compounds to be very satisfactory both when diluted with water and with oil. In an operation involving the drawing of bomb noses, the steel drew without wrinkling or breaking, and polishing of the die was not required during the entire test period.

An emulsion prepared from the lubricating composition of Example 1 performed satisfactorily in the drawing of rods from 0.75 inch to 0.63 inch.

It will be obvious to those skilled in the art that many modifications may be made within the scope of the present invention without departing from the spirit thereof, and the invention is to be restricted in accordance only with the appended claim.

We claim:

An emulsifiable lubricating composition comprising 60 to 75% by weight of a suspended phase consisting essentially of about 85 to 97% by weight of an inert solid material selected from the group consisting of calcium carbonate, zinc sulfide, lithopone, and talc having a hardness of 1 to 3.5 on Mohs' scale and a particle size at least fine enough to pass a 150 mesh screen and about 3 to

15% by weight of hydrophilic bentonite, and from about 40 to 25% by weight of a suspending phase consisting essentially of about 50 to 88% by weight of a mineral lubricating oil having a viscosity within the range of about 50 to about 500 SUS at 100° F. and about 12 to 50% by weight of an emulsifying agent of the oil-in-water type.

## References Cited in the file of this patent

## UNITED STATES PATENTS

|   |           |        |       |               |
|---|-----------|--------|-------|---------------|
| 5 | 1,739,631 | Cross  | ----- | Dec. 17, 1929 |
|   | 1,871,939 | Adams  | ----- | Aug. 16, 1932 |
|   | 2,210,177 | Rader  | ----- | Aug. 6, 1940  |
|   | 2,258,309 | Zimmer | ----- | Oct. 7, 1941  |
|   | 2,697,072 | Roden  | ----- | Dec. 14, 1954 |
|   | 2,722,515 | Reamer | ----- | Nov. 1, 1955  |
|   | 2,760,931 | Spring | ----- | Aug. 28, 1956 |